

Feb. 15, 1955

W. A. BIGGS, JR., ET AL

2,702,167

YARN PACKAGE

Filed Nov. 3, 1951

*Fig. 1*



*Fig. 2*



INVENTORS  
WILLIAM A. BIGGS, JR. &  
WILLIAM S. ADAMS  
BY

Panott, Richards & Sims  
ATTORNEYS

1

2,702,167

## YARN PACKAGE

William A. Biggs, Jr., and William S. Adams, Hartsville, S. C., assignors to Sonoco Products Company, a corporation of South Carolina

Application November 3, 1951, Serial No. 254,762

3 Claims. (Cl. 242—161)

This invention relates to textile yarn carriers, and in particular to a conical carrier having a specially adapted flock coating for handling multifilament yarns.

For many years, paper cones having a 3° 30' taper have been the standard carrier for synthetic textiles such as viscose, cuprammonium, acetate, Vinyon, nylon, etc. To obtain good holding properties for the yarn on this tapered cone surface and to assure good release properties on delivery, it has previously been proposed to invest the cone with a so-called "velvet surface" as disclosed in Dunlap Patents 1,634,492 and 2,219,836, and good results have been obtained in handling ordinary yarns with cones surfaced in this manner. This "velvet surface" is produced by high speed sanding of the paper cone surface with various grits of sandpaper to produce an irregular surface characterized by a "nap" of paper fibers tilted to a more or less erect position. The fundamental holding mechanism on this surface is the single paper fiber, varying mainly in length by the choice of the abrasive grit plus an inherent roughness in the surface produced by scratching, particularly on the coarser grits.

Now, with yarns of lower filament denier and/or twist, and particularly the fine multifilament synthetic yarns which are characteristically formed of filaments from about  $\frac{1}{6}$  to 6 denier size, and which have been used increasingly by the textile industry to a marked extent in recent years, the performance of the ground "velvet surface" has not always been consistent or satisfactory. There has been difficulty with this surface both from the standpoint of holding the finer yarns without slippage when coned and of allowing uniform delivery at high speed without excessive tension increases when the last layers of yarn on the surface are pulled away.

A mechanical analysis of the nature of the holding surface of a conical yarn carrier to illustrate the basic problem may be made in connection with the accompanying drawings in which:

Fig. 1 is a schematic diagram illustrating the relation of a yarn winding on a cone surface to a holding fiber; and

Fig. 2 is a schematic representation of yarn delivery tension test apparatus employed in developing the present invention.

If there is visualized a cylindrical fiber or yarn wrapped around a smooth, tapered cone surface under tension and at right angles to the long axis of the cone as indicated in Fig. 1, then the tendency  $S$  of the fiber to slip down the taper varies as the product of the winding tension  $T$  and the sine of the angle of taper  $\phi$ . At normal winding tensions, i. e.,  $\frac{1}{10}$  gm./denier, this slipping force  $S$  is relatively small and theoretically only a slight resistance in the holding surface would be required to hold it at the relatively low taper angle  $\phi$ . However, in practice and particularly with reciprocating winding, considerably more is required for safety.

Now, when the mechanism restraining the yarn from slippage on the cone taper is a more or less erect, single, essentially round holding fiber, then the restraining force  $F$  is equal to  $\pi$  times the elastic stiffness of the holding fiber material, times the fourth power of the fiber diameter  $d$ , divided by a constant times the radius of curvature of bending  $C$ , times the fiber length  $l$  to the point of application of the restraining force  $F$  (see Harold Dewitt Smith, "Textile Fibers, an Engineering Approach to Their Properties and Utilization," Edgar Marburg Lecture, 1944, ASTM, pp. 38-39), or,

2

$$F = \frac{\pi S g}{64 C l} \cdot d^4$$

5 where,

$F$ =restraining (or bending) force

$C$ =radius of bending

$l$ =bending length

10  $S$ =elastic stiffness of the holding fiber material  
 $d$ =holding fiber diameter

Since the wound fiber or yarn must be released on delivery without excessive tension increase in order to avoid breakage or stretch beyond the elastic limit which may result in "dye-resist" spots, the conical holding surface of the yarn carrier must be a carefully balanced compromise between the resistance or restraining force  $F$  needed for satisfactory holding in the package and that for allowing proper delivery. The ideal case would be where the restraining force  $F$  equaled the slipping force  $S$  and corresponded to the allowable tension on the wound fiber or yarn. This points up the shortcoming of the "velvet surface" obtained by grinding a paper cone, because grinding does not essentially alter the paper fiber diameter, so that the only variable available for altering surface properties, other than paper of different fiber size, is fiber length; and a study of the mechanics involved will show that altering the length will not effect the delivery materially for a given yarn without effecting the holding at the same time. As to papers composed of fibers of different diameters, the range is very limited. In addition, the age, source, and treatment of the same paper fibers may alter their inherent stiffness in a manner that is practically unpredictable.

35 With multifilament yarns of very low twist (0-2.5 turns) the problem is greatly complicated further because, at such twists, the yarn tends to behave not as a compact solid mass, but rather as a number of independent filaments flattening out more or less under tension against the holding surface. Under these conditions the tendency to slip may be less, due to greater contact area, but from a release standpoint the yarns are much more sensitive, since the filament diameters are very small as compared to the diameter of the yarn twisted from them.

40 Confronted with this problem, we have found that conical yarn carriers may be provided with a flock coating wherein the holding fibers on the cone surface are more or less erect, and which may be specially adapted for use with multifilament yarns on the basis of a definite relation for good delivery between the size and stiffness of the fiber holding and the size and twist of the yarn or fiber being held. Thus we have found that:

(1) The allowable holding fiber denier for good delivery at a given angle of held yarn twist varies as the square root of the held yarn denier.

(2) The allowable holding fiber denier for good delivery for a given held yarn of a given denier varies as the square of the sine of the angle of held yarn twist up to a twist angle of approximately  $10^\circ$ , above which the allowable holding fiber denier becomes essentially constant.

(3) The allowable stiffness of the holding fiber for good delivery of a given held yarn varies as the square of the holding fiber denier times the inherent dynamic stiffness of the holding fiber material at a given delivery speed, and which stiffness may be expressed in grams per denier.

70 By "good delivery" it is meant that the held yarn may be delivered directly from the flock coated cone surface at substantially the same tension at which it will deliver over itself from a wound package, or, in other words, that the inner windings of a yarn package supported on the flock coated cone surface will deliver without substantial variation from the tension employed to deliver the remaining or outer yarn windings from the yarn package.

75 The foregoing relations are demonstrated by the results outlined below of tests made to measure the effect of holding fibers of different diameters and stiffness on the delivery of yarns of different diameters and twist.

Flock surfaces were produced on smooth-finished paper cones in a variety of textures by application of flock cut from filaments of the following deniers:

TABLE 1

| Denier | Yarn    | Diameter (Microns) |
|--------|---------|--------------------|
| 0.75   | Viscose | 7.5                |
| 1.00   | do      | 9.6                |
| 1.50   | do      | 12.0               |
| 3.00   | do      | 16.7               |
| 5.50   | do      | 22.5               |
| 8.0    | Acetate | 29.1               |
| 12.0   | do      | 35.7               |
| 15.0   | Nylon   | 43.1               |
| 18.0   | Viscose | 40.9               |
| 50.0   | Nylon   | 78.0               |

These flocks were cut in a Sprout-Waldron revolving blade cutter taking the fraction passing a 60 mesh screen, or that which would yield fibers of varied length up to about 1 to 2 mm. in length. Application to the cone was made by spraying an aqueous flock adhesive on the cone followed by spraying on the flock from a De Vilbiss type flock gun. In each case the entire outer surface of the cone was heavily flocked except for an area one inch back from the nose which was left smooth.

In order to study delivery tensions, a typical creeling set-up was constructed with a wrapper and suitable instrumentation to obtain the tensions of delivery with precision. The creel was arranged for a single "end," and a simulated warp beam was provided by a carefully balanced 36-inch pulley equipped with a variable speed drive. The complete set-up is shown schematically in Fig. 2 of the drawings.

In Fig. 2, a  $3^\circ 30'$  cone is indicated at 10 carrying yarn windings that are being delivered as when the cone 10 is in position on the creel (not shown). At 20 a more or less conventional type of tensioning arrangement is indicated comprising a porcelain guide 21, a light tension disc 22 floating on the yarn and free to turn under friction and subject to added weight for tension control, and a molded plastic pulley 23 free to turn on a ball-bearing and resting on and turning against a felt washer for snubbing action, and to which weight might also be added for tension control, the yarn being looped completely around this pulley 23.

A tensiometer is indicated at 30 for giving dial readings of the tension, the yarn being looped around jewel bearing rollers 31 and 32 with the arm of roller 31 arranged to swing back and forth as the tension varies; and at 40 a phototensometer is represented comprising jewelled bearing rollers 41 and 42 and a sensing element 43, with the yarn threaded behind the rollers 41 and 42 and in front of the sensing element 43. This sensing element 43 reflects tension changes by oscillating slightly against a light helical spring 45, and the oscillation of sensing element 43 is picked up by a small mirror 44 arranged to swing or rock in accordance with the oscillation. A light beam from a lamp 46 is focused on the mirror 44 and is thereby angled to track on a light-sensitive film 47 travelling in front of it. Hence, any variation in yarn tension is recorded very sensitively by exposure of the film 47 and by varying the speed of the film travel very detailed recordings may be made of the delivery from one end of the cone traverse to the other.

Beyond the phototensometer a further porcelain guide 50 is arranged from which the yarn is taken onto the warp beam 60.

In operating this equipment, the following constant conditions were established.

Winding tension at  $\frac{1}{10}$  gram per denier of yarn,  $\pm 0.03$ ; Winding ratio at 2.5; Creeling tension at  $\frac{1}{10}$  gram per denier of yarn,  $\pm 0.03$ ; Creeling speed at 300 yards per minute; Cone taper at  $3^\circ 30'$ ; Cone length at  $6\frac{1}{4}$  inches; Flock density on surface as sprayed to excess; Ballooning angle fixed for a given yarn at fixed speed and tension; Oiling-run as supplied by yarn manufacturer;

and the following commercially available multifilament yarns were selected for test purposes:

TABLE 2

|    | Type    | Finish    | Denier | Filaments | Twist (turns/inch) |
|----|---------|-----------|--------|-----------|--------------------|
| 10 | Viscose | (Cordura) | 50     | 20        | 5.8                |
|    | Do      | Bright    | 75     | 30        | 2.1 Z              |
|    | Do      | do        | 75     | 30        | 4                  |
|    | Do      | do        | 75     | 30        | 10                 |
|    | Do      | do        | 75     | 30        | 15                 |
|    | Do      | do        | 75     | 30        | 20                 |
|    | Do      | do        | 75     | 30        | 38                 |
|    | Do      | do        | 75     | 30        | 49                 |
|    | Do      | do        | 100    | 40        | 2.1 S              |
|    | Do      | do        | 100    | 60        | 2.3 S              |
|    | Do      | do        | 100    | 60        | 5                  |
|    | Do      | do        | 100    | 60        | 10                 |
|    | Do      | do        | 100    | 60        | 18                 |
|    | Do      | Bright    | 125    | 50        | 2.5 S              |
|    | Do      | do        | 150    | 40        | 5                  |
|    | Do      | do        | 150    | 40        | 11                 |
|    | Do      | Dull      | 150    | 90        | 1.8 Z              |
|    | Do      | do        | 150    | 90        | 4                  |
|    | Do      | do        | 150    | 90        | 9.5                |
|    | Do      | do        | 150    | 90        | 21                 |
|    | Do      | Semi-Dull | 250    | 60        | 2.3 S              |
|    | Do      | Dull      | 300    | 50        | 2.5 S              |
|    | Do      | do        | 300    | 50        | 4                  |
|    | Do      | do        | 300    | 50        | 10                 |
|    | Do      | (Cordura) | 300    | 120       | 2.5 S              |
|    | Do      | do        | 300    | 120       | 10                 |
|    | Do      | Bright    | 450    | 72        | 2.5                |
|    | Do      | do        | 900    | 144       | 2.5                |

All yarns tested were coned on a #50 Universal Winder used exclusively for this purpose, and all work was done at 65% relative humidity and 70° F., so that the operating conditions substantially isolated the two important variables of holding flock denier and held yarn denier to be studied against each other at various twists with varying filament numbers and finishes.

In making the tests approximately 300 yards of each yarn was wound on a test cone, leaving several yards of "pigtail." Before delivery the pigtail was removed from the cone base so that it could be delivered as a free end and thereby avoid any masking of the effect of the cone surface at the critical point of the run-out.

As a criterion for surface evaluation, the standard "good" was chosen for the maximum holding flock denier from which a given held yarn could be delivered without essential increase in tension variation at the final runout over the variation existing with the yarn running over itself; the next highest holding flock denier from which the held yarn could not be delivered under these conditions was taken as "bad." Due to the gaps between the denier of flock available for study, points of maximum tolerance could not be finely established, so that a range for "good" delivery and "bad" delivery is reported in each case. The test results are presented in Table 3 under the heading "Flock denier (FD)" with observed values for "good and "bad":

TABLE 3

65 The effect of twist and denier of held yarn on delivery from various denier of flock surfaced  $3^\circ 30'$  cones

| Viscose Yarn | Twist | Flock Denier (FD) |     |
|--------------|-------|-------------------|-----|
|              |       | Good              | Bad |
| 50/20        | 5     | 1.5               | 8   |
| 75/30        | 2.1   | 0.75              | 1   |
| 75/30        | 4     | 1.5               | 8   |
| 75/30        | 10    | 8                 | 12  |
| 75/30        | 15    | 8                 | 12  |
| 75/30        | 20    | 8                 | 12  |
| 75/30        | 38    | 8                 | 12  |
| 75/30        | 49    | 8                 | 12  |
| 75/30        | 2.5   | 1.5               | 8   |
| 100/40       | 2.3   | 1.5               | 8   |
| 100/60       | 5     | 8                 | 12  |
| 100/60       | 9.5   | 8                 | 12  |
| 100/60       | 18    | 8                 | 12  |
| 125/60       | 2.4   | 1.5               | 8   |
| 150/40       | 2.5   | 8                 | 12  |
| 150/40       | 5.25  | 12                | 15  |
| 150/40       | 11    | 12                | 15  |
| 150/40       | 22    | 12                | 15  |

5  
TABLE 3—Continued.

| Viscose Yarn | Twist | Flock Denier (FD) |     |
|--------------|-------|-------------------|-----|
|              |       | Good              | Bad |
| 160/60       |       | 1.8               | 1.4 |
| 160/60       | 4     | 3                 | 5.5 |
| 150/60       | 9.5   | 12                | 18  |
| 150/60       | 21    | 12                | 18  |
| 260/60       | 2.5   | 8                 | 18  |
| 300/60       | 2.5   | 8                 | 18  |
| 300/60       | 4     | 12                | 18  |
| 300/60       | 10    | 18                | 50  |
| 300/120      | 2.5   | 8                 | 4.5 |
| 300/120      | 10    | 18                | 18  |
| 450/72       | 2.5   | 12                | 18  |
| 500/144      | 2.5   | 18                | 30  |

Examination of these data point up the obvious fact that increasing the twist in a given held yarn increases its resistance to snagging and consequently its tolerance for stiffer holding fibers or flock very markedly, although at higher twists improvement in tolerance levels off. Also, the tolerance for stiffer holding fibers increases with the denier of the held yarn being delivered, and held yarns made up of more and smaller filaments at low twist have less tolerance than an equivalent denier yarn composed of larger filaments.

Analysis of these data further reveal that if the allowable holding flock denier for 75/30 yarn, for example, is plotted against the twist angle, or its tangent calculated in accordance with Milton M. Platt, "Mechanics of elastic performance of textile materials," Textile Research Journal, 20, p. 3 (January 1950), for each twist number, then a fairly smooth S type curve is obtained which corresponds almost exactly with a  $\sin^2$  curve plotted for the twist angle  $\theta$ , and from which correspondence the following relation can be derived:

$$FD_{75} = 10 \sin^2 (500 \tan \theta)$$

where  $FD_{75}$  is the allowable holding flock denier for good delivery of 75 denier held yarn; and  $\tan \theta$  is equal to or less than 0.18, since there is no further improvement in delivery above the twist angle  $\theta$  (approximately 10°) at which  $\tan \theta$  becomes 0.18.

Using this relation, the theoretical allowable holding flock deniers were calculated and recorded against the observed values for a typical group of the 75/30 yarns under consideration, and the results are shown in Table 4 below:

TABLE 4

| Yarn  | Twist | Average Dia. (") | $\theta^{\circ}$ | Tan $\theta$ | FD         |           |
|-------|-------|------------------|------------------|--------------|------------|-----------|
|       |       |                  |                  |              | Calculated | Observed  |
| 75/30 | 2.1   | .00467           | 1.78             | .0908        | 0.71       | 0.75 to 1 |
| 75/30 | 4     | .00448           | 3.21             | .0563        | 2.23       | 1.5 to 8  |
| 75/30 | 10    | .00430           | 7.70             | .1350        | 8.58       | 8.0 to 12 |
| 75/30 | 38    | .00379           | 24.37            | .4827        | 10.00      | 8.0 to 12 |
| 75/30 | 49    | .00378           | 20.87            | .5742        | 10.00      | 8.0 to 12 |

It will be noted that the two sets of values check quite well as to range especially when it is realized that the calculated value is greatly dependent on precision measurement of the yarn diameter which necessarily depended upon the assumption that a microscopically examined sample was representative of several hundred yards of yarn. The impressive thing to consider from these results is the great dependence of the yarn behavior on the twist angle  $\theta$ , which not only reflects the twist in terms per inch but the yarn diameter as well.

To translate this twist angle-holding flock denier relation into a general one covering different deniers of held yarn, the above equation for allowable holding flock denier with 75 denier held yarn was stated in general form, i. e.:

$$FD = K \sin^2 (500 \tan \theta)$$

and was solved for  $K$  by inserting the experimental data for the yarns tested as tabulated below (Table 5), the

mean FD value for each yarn being used, and the results for each yarn denier being averaged:

6  
TABLE 5

| 5       | Yarn  | Twist | $\sin^2 (500 \tan \theta)$ | Average FD | K    | K Average |
|---------|-------|-------|----------------------------|------------|------|-----------|
| 10      | 50/20 | 5     | .219                       | 2.25       | 10.3 | 10.3      |
| 75/30   | 2.1   | .071  | .088                       | 12.4       |      |           |
| 75/30   | 4     | .202  | .235                       | 10.2       |      |           |
| 75/30   | 10    | .053  | .10.00                     | 11.7       |      |           |
| 75/30   | 25    | .001  | .00.00                     | 10.0       |      |           |
| 75/30   | 49    | .001  | .00.00                     | 10.0       |      |           |
| 100/40  | 2.5   | .131  | .225                       | 17.1       |      |           |
| 100/60  | 2.8   | .107  | .225                       | 20.9       |      |           |
| 100/60  | 5     | .339  | .425                       | 12.5       |      |           |
| 100/60  | 9.5   | .865  | .10.0                      | 11.7       |      |           |
| 125/60  | 3.4   | .134  | .225                       | 10.8       |      |           |
| 180/40  | 2.5   | .275  | .425                       | 15.4       |      |           |
| 180/40  | 54    | .741  | .13.5                      | 15.2       |      |           |
| 180/40  | 22    | 1.0   | .19.5                      | 16.5       |      |           |
| 180/40  | 1.8   | .166  | .225                       | 14.5       |      |           |
| 180/40  | 4     | .476  | .425                       | 4.5        |      |           |
| 180/40  | 9.5   | .896  | .13.5                      | 13.5       |      |           |
| 225/60  | 2.5   | .441  | .18.0                      | 22.7       |      |           |
| 300/40  | 2.5   | .442  | .10.0                      | 22.4       |      |           |
| 300/60  | 4     | .727  | .13.5                      | 18.5       |      |           |
| 300/60  | 10    | 1.0   | .20.0                      | 20.0       |      |           |
| 300/120 | 2.5   | .376  | .425                       | 11.5       |      |           |
| 300/120 | 10    | 1.0   | .13.5                      | 14.5       |      |           |
| 450/72  | 2.5   | .679  | .13.5                      | 22.3       |      |           |

Examination of the above data shows  $K$  to be varying roughly as the square root of the held yarn denier  $YD$ , which relation can be expressed as:

$$K = k \sqrt{YD}$$

where  $k$  is a constant dependent on the basic holding flock material and the conditions of delivery, so that the general relation for allowable holding flock denier FD then becomes:

$$FD = k \sqrt{YD} \sin^2 (500 \tan \theta)$$

Now, although this relationship is expressed generally in terms of the holding flock denier FD, it is obvious that the basic difference in the holding flock fibers of different denier which influences delivery performance of a given held yarn is the difference in relative dynamic stiffness; that is, the fiber stiffness at high loading rates, such as at the withdrawal or creeling speed of 300 yards per minute used in this investigation. That various types of fibers have different inherent stiffness properties that form an important factor in their performance as textile materials is well known, so that it was recognized that this factor should be accounted for too.

For this purpose, the relation (from Smith, above) of the stiffness of a cylindrical fiber as varying with the fourth power of the fiber diameter, or the square of its denier, may be employed by stating this relation as follows:

$$FS = Sd^4 = S_i FD^2$$

where  $FS$  is the holding flock stiffness; and  $S_i$  is the instantaneous or dynamic elastic stiffness of the flock in grams per denier.

This relation may then be stated as:

$$FD = \sqrt{\frac{FS}{S_i}}$$

and since

$$FD = k \sqrt{YD} \sin^2 (500 \tan \theta)$$

70 then

$$\sqrt{\frac{FS}{S_i}} = k \sqrt{YD} \sin^2 (500 \tan \theta)$$

75 and

$$FS = S_i [k \sqrt{YD} \sin^2 (500 \tan \theta)]^2$$

which places the relation of the denier of the held yarn and its twist to the holding flock in terms of the dynamic elastic stiffness of the holding flock to indicate the proportionate change for good delivery tolerance in holding flock of a given denier but different stiffness, or in different denier for a given stiffness.

The foregoing relations require the determination of a value for the constant  $k$  to match the properties of the

yarns being considered and the particular conditions of delivery, such as delivery speed, winding speed, carrier shape, etc., but otherwise they are fundamental in regard to the holding flock surface and state relations which allow the special adaption of flock coated yarn carriers for particularly effective and efficient handling of multi-filament yarns.

In addition, it should be noted that the relation derived above for holding flock stiffness  $FS$  states a basic relation that may be applied in handling all types of yarn on any shape of end delivery carrier, subject to suitable modification of the constant  $k$  for the particular case involved. A practical problem of holding and delivery exists even with parallel tube carriers for there is always a tendency of the yarn package to shift under impact, and the delivery problem is in fact more acute when a parallel tube core is used because there is no taper to facilitate the yarn release at run out when the yarn windings are being withdrawn directly from the carrier surface. As the angle of carrier taper increases, the holding problem likewise increases and the delivery problem decreases; while with a decreasing angle of taper, it is the delivery problem that increases, although the holding problem decreases. In any case, however, the fundamental relative behavior of the holding flock surface with various yarns remains essentially unaltered as established by the present invention.

The present invention has been described in detail above for purposes of illustration only and is not intended to be limited by this description or otherwise except as defined in the appended claims.

We claim:

1. A textile yarn package comprising yarn wound in package form on a supporting core having a winding surface retaining the inner windings of said yarn package against slippage thereon while allowing said inner windings to be delivered continuously and completely therefrom without essential increase in delivery tension over that existing when the yarn windings are delivering over themselves from the package, said winding surface being covered for this purpose with an adhesively secured flock coating, the flock forming said coating being composed of discrete fibers having an individual dynamic stiffness determined by the following relation:

$$FS = S_i [k \sqrt{YD} \sin^2 (500 \tan \theta)]^2$$

where  $FS$  is the flock stiffness;  $S_i$  is the instantaneous or dynamic elastic stiffness of the flock fiber in grams per denier;  $k$  is a constant for the particular delivered yarn fiber material and conditions of delivery;  $YD$  is the delivered yarn denier; and  $\theta$  is the twist angle of the delivered yarn up to the angle at which  $\tan \theta$  becomes 0.18.

5. 2. A textile yarn package as defined in claim 1 and further characterized in that said package comprises continuous filament yarn wound in package form.

10. 3. A textile yarn package comprising yarn wound in package form on a supporting core having a winding surface retaining the inner windings of said yarn package against slippage thereon while allowing said inner windings to be delivered continuously and completely therefrom without essential increase in delivery tension over that existing when the yarn windings are delivering over themselves from the package, said winding surface being covered for this purpose with an adhesively secured flock coating, the flock forming said coating being composed of discrete fibers having an inherent unit stiffness of the order of that of viscose fibers, and said flock fibers having an individual denier determined by the following relation:

$$FD = K \sqrt{YD} \sin^2 (500 \tan \theta)$$

15. where  $FD$  is the individual flock denier;  $K$  is a constant for the particular delivered yarn fiber material and conditions of delivery;  $YD$  is the delivered yarn denier; and  $\theta$  is the twist angle of the delivered yarn up to the angle at which  $\tan \theta$  becomes 0.18.

20. 35. References Cited in the file of this patent

UNITED STATES PATENTS

|           |           |       |               |
|-----------|-----------|-------|---------------|
| 2,076,451 | Fallsheer | ----- | Apr. 6, 1937  |
| 2,219,836 | Dunlap    | ----- | Oct. 29, 1940 |
| 2,430,710 | Dunlap    | ----- | Nov. 11, 1947 |

40. FOREIGN PATENTS

|     |               |       |              |
|-----|---------------|-------|--------------|
| 885 | Great Britain | ----- | Mar. 5, 1879 |
|-----|---------------|-------|--------------|

UNITED STATES PATENT OFFICE  
CERTIFICATE OF CORRECTION

Patent No. 2,702,167

February 15, 1955

William A. Biggs, Jr., et al.

It is hereby certified that error appears in the printed specification of the above numbered patent requiring correction and that the said Letters Patent should read as corrected below.

Column 3, line 31, for "wrapper" read --warper--; line 38, for "3° 3°", read --3° 30'--; column 4, line 60, for '"good' read --"good"--; column 6, Table 5, third column, 12th line thereof, for "2.76" read --.276--; line 35, for "reation" read --relation--.

Signed and sealed this 22nd day of March, 1955.

(SEAL)

Attest:

E. J. MURRY

Attesting Officer

ROBERT C. WATSON  
Commissioner of Patents